

# United States Patent Office

2,985,529  
Patented May 23, 1961

1

2,985,529

## CREEP RESISTANT NON-AUSTENITIC STEELS

Geoffrey T. Harris, Sheffield, and Henry C. Child, Rotherham, England, assignors to The Birmingham Small Arms Company Limited, Birmingham, England, a company of Great Britain

No Drawing. Filed Aug. 24, 1959, Ser. No. 835,415

Claims priority, application Great Britain Aug. 27, 1958

9 Claims. (Cl. 75—126)

This invention relates to ferritic or martensitic (i.e., non-austenitic) chromium alloy steels of the kind intended for use at high temperatures, i.e., of the order of 600–700° C.

Such alloy steels have been used to a large extent in recent years for creep-resistance applications, but there is a continual demand for improved creep-strength.

Examples of developments in this field are to be found in British Patents Nos. 638,110; 658,115; 730,272; 733,146 and 796,733. In these patents alloys are disclosed containing from about 9% to about 20% chromium and, in

The following is a preferred narrower range of elements according to the invention any one or all of which may be substituted for the corresponding element or elements in the ranges given above:

|                            | Percent              |
|----------------------------|----------------------|
| Carbon                     | 0.08–0.2             |
| Nickel                     | 0–2                  |
| Chromium                   | 10–13                |
| Cobalt                     | 5–10                 |
| Tungsten and/or molybdenum | 0–2                  |
| Niobium and/or tantalum    | <sup>1</sup> 1.5–2.5 |
| Vanadium                   | 0–1.5                |
| Boron                      | 0–0.02               |
| Nitrogen                   | .02–0.09             |
| Aluminium                  | 0–0.1                |

<sup>1</sup> Must be in excess of tungsten and/or molybdenum.

Preferably the total of tungsten or molybdenum is below 1% and, still more preferably, below 0.5%.

Where no intentional nitrogen addition has been made, additions of the deoxidiser, zirconium, are desirable in amounts of up to 0.2%.

The following examples illustrate the invention, the alloy W. 684 not being in accordance with the present invention but being inserted for purposes of comparison:

|        | C    | Mn  | Si  | Ni  | Cr   | Co | W   | Mo  | V    | Nb   | B    | N    |
|--------|------|-----|-----|-----|------|----|-----|-----|------|------|------|------|
| W. 684 | 0.13 | 1.2 | 0.3 | 0.8 | 10.5 | 5  | 1.0 | 1.0 | 0.5  | 0.5  | 0.01 | 0.07 |
| W. 857 | 0.15 | 1.2 | 0.3 | 0.8 | 10.5 | 5  | 0.4 | 0.4 |      | 2.2  | 0.01 | 0.07 |
| W. 862 | 0.12 | 1.2 | 0.3 | 0.8 | 10.5 | 5  | 0.4 | 0.4 | 0.35 | 1.85 | 0.01 | 0.07 |
| W. 866 | 0.15 | 1.2 | 0.3 | 0.8 | 10.5 | 5  | 0.4 | 0.4 | 1.5  | 1.5  | 0.01 | 0.07 |

addition, one or more of molybdenum, tungsten, vanadium, niobium, tantalum or titanium. As deoxidisers manganese and silicon are usually added. Nickel may also be incorporated, usually in amounts up to about 5%. For most practical purposes it is desirable that the carbon content should be below about 0.3%.

In the prior work little, if any, attention has been given to the relationship between tungsten and/or molybdenum on the one hand and niobium and/or tantalum on the other hand. Whilst not advancing any particular theory, we have found, and this forms the basis of the present invention, that in alloys of the kind in question improved creep strength may be obtained if the content of niobium and/or tantalum exceeds the content of tungsten and/or molybdenum and the latter may be omitted entirely. Further, in much of the work in this field, vanadium has been regarded as an essential alloying constituent. Alloys according to the present invention need not necessarily contain vanadium. Nickel may also be omitted. According to a feature of this invention alloy steels of the kind referred to comprise the following ingredients within the ranges specified, the percentages being by weight:

|                            | Percent          |
|----------------------------|------------------|
| Carbon                     | 0.01–0.2         |
| Nickel                     | 0–4              |
| Chromium                   | 9–15             |
| Cobalt                     | 3–15             |
| Tungsten and/or molybdenum | 0–2              |
| Niobium and/or tantalum    | <sup>1</sup> 1–3 |
| Vanadium                   | 0–3              |
| Boron                      | 0–0.5            |
| Nitrogen                   | 0–0.1            |
| Aluminium                  | 0–0.1            |

<sup>1</sup> Must be in excess of tungsten and/or molybdenum.

together with deoxidisers, e.g., manganese 0.1–2% and silicon 0.1–1%, and iron and impurities which form the balance.

35 In each of these alloys iron and impurities constituted the balance. When tested at 8 tons at 600° C. these four alloys reached the total plastic strain in 100 hours indicated below:

|        | Percent |
|--------|---------|
| W. 684 | .1      |
| W. 857 | .06     |
| W. 862 | .038    |
| W. 866 | .04     |

45 These tests were carried out with material oil-quenched from 1200° C. and tempered at 650° C.

It was found that still further improvements could be achieved by tempering at higher temperatures, e.g., by tempering at 700° C. The creep strength of W. 862 based on a criterion of 0.1% total plastic strain in 100 hours at 600° C. was 23 tons/sq. in. This might be compared with similar creep strength of 10 tons/sq. in. for W. 684.

55 Satisfactory creep strengths which would be acceptable for many purposes, however, could be obtained by solution treating over a wide range of temperatures from 1000° C. to 1250° C. and tempering in the range 550° to 750° C.

The influence on the creep strength, of some of the various alloying additions, is tabulated below.

The basic alloy was W. 862, the composition of which is given above.

The composition of the alloys was kept to this specification, except, of course, for the element which was being varied.

65 In order to indicate the effect of heat treatment, two results are given for some alloys, one in heat treated Condition A and the other in Condition B or C.

70 Condition A: ½ hr. at 1200° C., oil quenched, 2 hrs. at 650° C., air cooled.

## Condition B:

½ hr. at 1200° C., oil quenched,  
2 hrs. at 700° C., air cooled.

## Condition C:

½ hr. at 1200° C., oil quenched,  
2 hrs. at 725° C., air cooled.

## Effect of niobium tantalum

[Stress to give 0.1% in 100 hours at 600° C.]

| Alloy | Percent<br>Nb | Stress in tons/sq. in. |    | 15 | 15 |  |  |
|-------|---------------|------------------------|----|----|----|--|--|
|       |               |                        |    |    |    |  |  |
|       |               | A                      | C  |    |    |  |  |
| 1     | 1.5           |                        |    | 15 |    |  |  |
| 2     | 1.7           | 16                     | 22 |    |    |  |  |

## Effect of cobalt

[Stress to give 0.1% in 100 hours at 600° C.]

| Alloy | Percent<br>Co | Stress in tons/sq. in. |   | 23 | 28 |
|-------|---------------|------------------------|---|----|----|
|       |               | A                      | B |    |    |
| 2     | 5             | 15                     |   | 23 |    |
| 3     | 7             | 20                     |   |    | 28 |
| 4     | 10            | 12                     |   |    | 15 |

## Effect of the ratio of the carbide formers when total kept at 3%

[Tested under 17 tons/sq. in. at 600° C.]

| Alloy | Nb,<br>percent | V,<br>percent | Mo+W,<br>percent | Percent strain<br>in 100 hours |      |
|-------|----------------|---------------|------------------|--------------------------------|------|
|       |                |               |                  | A                              | B    |
| 10    | 2.52           |               | 0.48             | 0.32                           | 0.23 |
| 13    | 2.33           | 0.32          | 0.48             | 0.27                           | 0.20 |
| 14    | 1.90           | 0.62          | 0.49             | 0.15                           | 0.11 |
| 15    | 2.2            |               | 0.8              | 0.20                           | 0.10 |
| 2     | 1.75           | 0.28          | 0.85             | 0.15                           | 0.06 |
| 16    | 1.5            | 0.7           | 0.8              | 0.32                           | 0.50 |
| 17    | 1.98           | 0.17          | 1.07             | 0.12                           | 0.06 |

It may be seen that whilst a small addition of vanadium has a beneficial effect on the creep strength at 600° C., the properties of the vanadium free alloy 15 still show a substantial improvement over previous alloys with low niobium content. It is also evident that a high tungsten and molybdenum content is beneficial, although, of course, this content still remains lower than the total content of niobium and tantalum.

The following are examples of alloy steels according to the invention in which tungsten and molybdenum are absent the alloy W. 954 (not being according to the invention) being included for the purposes of comparison:

|        | C    | Mn  | Si  | Ni  | Cr   | Co  | V   | Nb  | Al   | B    | N        | Fe and<br>impuri-<br>ties |
|--------|------|-----|-----|-----|------|-----|-----|-----|------|------|----------|---------------------------|
| W. 954 | 0.12 | 1.2 | 0.3 | 0.8 | 10.5 | 5.0 | 3.0 | 0.1 | 0.01 | 0.07 | Balance. |                           |
| W. 955 | 0.12 | 1.2 | 0.3 | 0.8 | 10.5 | 5.0 | 3.0 | 0.1 | 0.01 | 0.07 | Do.      |                           |
| W. 956 | 0.12 | 1.2 | 0.3 | 0.8 | 10.5 | 5.0 | 1.5 | 0.1 | 0.01 | 0.07 | Do.      |                           |

## Effect of carbon on alloys containing 7% Co

[Tested under 20 tons/sq. in. at 600° C.]

| Alloy | Percent<br>C | Percent strain in<br>100 hours |       | 40 |
|-------|--------------|--------------------------------|-------|----|
|       |              | A                              | B     |    |
| 3     | 0.13         | 0.10                           | 0.065 |    |
| 5     | 0.10         | 0.29                           | 0.28  |    |
| 6     | 0.08         | 0.53                           | 0.35  |    |

## Effect of boron

[Tested under 20 tons/sq. in. at 600° C.]

| Alloy | Percent<br>B | Percent strain in<br>100 hours |      | 50 |
|-------|--------------|--------------------------------|------|----|
|       |              | A                              | B    |    |
| 7     | 0.0009       | 0.85                           | 1.0  |    |
| 8     | 0.005        | 0.37                           | 0.26 |    |
| 2     | 0.01         | 0.25                           | 0.07 |    |
| 9     | 0.019        | 0.13                           | 0.09 |    |
| 10    | 0.045        | 0.13                           | 0.17 |    |

## Effect of nitrogen

[Tested under 20 tons/sq. in., at 600° C.]

| Alloy | Percent<br>N | Percent strain in<br>100 hours |      | 70 |
|-------|--------------|--------------------------------|------|----|
|       |              | A                              | B    |    |
| 11    | 0.013        | 0.46                           | 0.50 |    |
| 2     | 0.075        | 0.25                           | 0.07 |    |

## Creep strengths

## Heat treatment:

½ hr. at 1200° C., oil quenched

2 hrs. at 650° C., air cooled

Testing: 8 tons/sq. in., at 600° C.

|        | Time to<br>0.05%,<br>hrs. | Time to<br>0.1%,<br>hrs. | Strain,<br>percent<br>in 100<br>hours |
|--------|---------------------------|--------------------------|---------------------------------------|
| W. 954 |                           |                          | 34                                    |
| W. 955 |                           | 112                      | 1.0                                   |
| W. 956 |                           | 14                       | 0.05                                  |
|        |                           | 67                       | 0.12                                  |

The alloys of the invention may be contrasted with martensitic alloys having roughly the same chromium content but with low niobium proportions. Examples of such alloys are:

|                   | Percent | Percent |
|-------------------|---------|---------|
| 60 C              |         | 0.16    |
| Mn                |         | 0.7     |
| Si                |         | 0.3     |
| Ni                |         | 0.24    |
| Cr                | 11.6    | 10.5    |
| Mo                | 0.6     | 0.8     |
| W                 |         | 0.8     |
| Nb                | 0.25    | 0.45    |
| Co                |         | 6.7     |
| V                 | 0.3     | 0.55    |
| Fe and impurities |         | Balance |

These alloys have a creep strength at 600° C. based on 0.1% total plastic strain in 100 hours of approximately 9 tons. Also, when tested at 20 tons at 600° C. they reach a plastic strain of more than 1% in 100 hours and fracture at approximately 150 hours. It will be seen, therefore, that alloys according to the present invention are significant improvements on these earlier alloys.

We claim:

1. Non-austenitic alloy steels consisting by weight essentially of 0.01 to 0.2% carbon, nickel up to 4%, chromium 9-15%, cobalt 3-15%, one or more materials selected from the group consisting of tungsten and molybdenum up to 2%, one or more materials selected from the group consisting of niobium and tantalum 1-3% and in excess of the total material or materials selected from the group consisting of tungsten and molybdenum, vanadium up to 3%, boron up to 0.05%, nitrogen up to 0.1%, aluminium up to 0.1%, and the balance essentially iron.

2. Alloy steels according to claim 1 in which up to 2% vanadium is present.

3. Alloy steels according to claim 1 containing one or more materials from the group consisting of manganese and silicon, said manganese being present within the range of 0.1 to 2%, and said silicon being present in the range of 0.1 to 1%.

4. Alloys according to claim 1 in which the tungsten content is less than 1%.

5. Alloy steels according to claim 1 in which the tungsten content is less than 0.5%.

6. Alloy steels according to claim 1 in which the molybdenum content is less than 1%.

7. Alloy steels according to claim 1 in which the molybdenum content is less than 0.5%.

8. Non-austenitic alloy steels consisting by weight essentially of 0.08 to 0.2% carbon, nickel up to 2%, chromium 10-13%, cobalt 5-10%, one or more materials selected from the group consisting of tungsten and molybdenum up to 2%, one or more materials selected from the group consisting of niobium and tantalum 1.5 to 2.5% and in excess of the total material or materials selected from the group consisting of tungsten and molybdenum, vanadium up to 1.5%, boron up to 0.02%, nitrogen 0.02 to 0.09%, aluminium up to 0.1%, and the balance essentially iron.

9. Non-austenitic alloy steels consisting by weight essentially of 0.01 to 0.2% carbon, nickel up to 4%, chromium 9-15%, cobalt 3-15%, one or more materials selected from the group consisting of tungsten and molybdenum up to 2%, one or more materials selected from the group consisting of niobium and tantalum 1-3% and in excess of the total material or materials selected from the group consisting of tungsten and molybdenum, vanadium up to 3%, boron up to 0.05%, aluminium up to 0.1%, and the balance essentially iron with up to 0.2% zirconium as a deoxidiser.

References Cited in the file of this patent

UNITED STATES PATENTS

1,711,484 Armstrong ----- May 7, 1929